

June 6, 1967

D. STRAW ET AL

3,323,917

PHOTOMECHANICAL BLEACHOUT COLOR PROCESS

Filed March 7, 1963



FIG. 1



FIG. 2



FIG. 3



FIG. 4



FIG. 5



FIG. 6



FIG. 7

INVENTORS

DOUGLAS STRAW  
CLIFFORD E. HERRICK, JR.

BY

*Henry W. Coughlin*  
*Edward P. Gilkerson*

ATTORNEYS

1

3,323,917  
**PHOTOMECHANICAL BLEACHOUT COLOR  
PROCESS**

Douglas Straw, Binghamton, N.Y., and Clifford E. Her-  
rick, Jr., Concord, Mass., assignors to General Aniline  
& Film Corporation, New York, N.Y., a corporation of  
Delaware

Filed Mar. 7, 1963, Ser. No. 263,563  
4 Claims. (Cl. 96—27)

The present invention relates to a photomechanical bleachout color process. It has particular application to a positive working photomechanical bleachout process which is capable of yielding high-contrast images in a number of colors.

A widely used, modern technique in color reproduction is the diazotype system, which involves the use of a so-called intermediate. In place of making a large number of copies from a frail and valuable original, it is customary to make a single copy on an intermediate material or support. From this, additional prints, can be made.

A thin material, such as a foil, is frequently used and in order to be satisfactory as an intermediate material, this should have the fastest possible printing speed consistent with good opacity. It should be stabilized against precoupling, or yellowing, or offsetting tendencies. A very satisfactory product of this type has been disclosed in application Ser. No. 641,023 filed Feb. 19, 1957 now Patent No. 2,940,852. Materials of the type disclosed in this application satisfy many of the requirements, but they frequently suffer from slow printing speeds and yield prints of only mediocre to fair contrast.

These properties of slow printing speeds and inadequate contrast are particularly disadvantageous in graphic art applications. In these, printing exposures are necessarily made under a vacuum contact with an arc lamp in order to insure good resolution. These devices require considerable exposure time, as much as several minutes. The amount of light-sensitive material present in the light-sensitive layer or the amount of material photodecomposed therein is directly related to the image density. Also, although the contrast of diazotype materials is normally considered quite good in comparison to conventional silver halide photographs, it is only marginally acceptable in certain graphic art applications where there is a higher requirement for contrast.

Diazotype foils, or intermediates which are capable of bearing images in different colors, are used for the pre-testing and proofing of half-tone color separation positives. Such materials are used in the production of color printing plates for offset, letterpress or gravure printing. It is well known that such positive half-tone color separation films, or plates, normally require a certain amount of hand correction. In other words, they must be touched up to reproduce faithfully the colors of the original subject or scene in terms of printing press inks. Certain foils sold under the name "Ozachrome" have proved to be very helpful as a guide in such correction work. These foils are manufactured in colors which match to a rather high degree, the inks which are widely used in printing. The particular shades, lightness or strengths of the inks can be matched by uniformly reducing the density of the whole sheet or foil by preflashing each of the several colors to a suitable level of density. This level, of course, may be different for different colors. Hence, each of the separation positives, which may be corrected by hand, frequently is printed onto a foil of the desired color. The Ozachrome foil of the prior art may be used and may be overlaid in register over a white background to produce the desired proof.

2

The printing process just described has its limitations, but has proved useful and, in fact, is used quite widely. The colors of the foils are determined by the manufacturer, depending upon the type of coating provided by him. Since the process inks are available in a very great variety of colors, it is usually impossible to achieve an exact color match between Ozachrome color, which is limited in variety and the inks used by the manufacturer. Furthermore, the prints made on diazotype foils often show discolored backgrounds. These may be caused either by premature coupling of the dye-forming components prior to processing and/or by discoloration of other ingredients such as the stabilizing chemicals after processing. These discolorations are very apparent in applications where two or more foils are laid over one another to produce a multicolor effect.

The present invention is designed to overcome some of these difficulties. It makes available a positive working process which is suitable for use on certain carrier layers having a reasonably high degree of light sensitivity. It is usable, moreover, in ordinary room illumination.

It is a further object of this invention to make available a good method whereby the color, or colors, used in making positive prints can be matched very exactly to a predetermined standard, both in density and in hue.

A still further object is to provide a high contrast, high resolution, and grainless copying media of very high printing speed. The image density, unlike the diazotype, is not explicitly related to the amount of light-sensitive material present in, or photodecomposed in, the light-sensitive layer. Hence, images of high visual and actinic opacity can be produced without sacrificing printing speed.

The new process of this invention is a direct copying method. It yields positive images from positive originals. Furthermore, the choice of primary and individual colors is practically unlimited.

The process of this invention, therefore, employs a layer of a compatible mixture of two major ingredients. One is a copolymer formed from about 1 mole of methylvinyl ether and 1 mole of maleic anhydride. This is referred to for brevity as PVM/MA. The other ingredient is some other hydrophobic resin or mixture of resins. This layer, composed of these major ingredients, may be called the carrier layer. The carrier layer may be hydrolyzed and rendered hydrophilic by any suitable process, for example, the process described in U.S. Patent 2,756,163. It may be subsequently dyed or the dyeing and hydrolyzing operations may be combined into a single operation by obtaining a solution of a dye in the hydrolyzing material. The dyes are selected to yield the proper hue and the dye density can be readily controlled by the dyeing time or the dye concentration, or by both. Dyes which are found to be suitable for this purpose include: Color Index Basic Yellow 1, 2, 4, 10, 11; Color Index Basic Orange 14, 22; Color Index Basic Red 1, 2, 5, 9, 13; Color Index Basic Violet 1, 3, 4, 5, 7, 10, 14; Color Index Basic Blue 1, 5, 6, 9, 12 and Color Index Basic Green 1, 4.

Still another scheme by which the carrier layer may be dyed, consists of forming an azo dye, or a plurality of azo dyes, in situ in the carrier layer. This may be accomplished by impregnating the carrier layer with the dye-forming components (diazot) and coupler and subsequently rendering the system alkaline, whereupon the dye forms. Among those diazonium compounds which have been found to be suitable for this purpose, mention may be made of the following diazotized amines; ortho-anisidine; 2,6-dimethoxyaniline; 2,4-dimethoxyaniline; orthophenetidine; 3,3'-dimethoxy-4,4'-diaminobiphenyl; 2-chloro-5-trifluoromethylaniline; 2-hydroxy-4-methyl-7-aminoquinoline; 4-aminobiphenyl; N,N'-diethylamine - para-phenylenediamine; 4-(N,N-diethylamino)-2-ethoxy - aniline; 4-(N,N-diethylamino)-2-methylaniline; 4-ethylami-

no-3-methylaniline; and the like. Among those coupling compounds which we have found to be suitable, mention may be made of: beta-naphthol-3,6-disulfonic acid; 2,7-dihydroxynaphthalene; 2,3-dihydroxynaphthalene; 2,3-dihydroxynaphthalene-6-sulfonic acid; phenylmethyl pyrazolone; phloroglucinol; 5,5-dimethyl-1,3-cyclo-hexanedi-one; m-hydroxyphenylurea, 7-hydroxy-1,2-naphthimidazole; resorcinol; 4,6-dichlororesorcinol, resorcinol sulfonic acid; and the like. Ammonia fumes have been found to be particularly suitable for rendering the system alkaline.

The carrier layer is then sensitized by coating it with a solvent solution containing the light-sensitive sensitizer. Sensitizers which have been found to be suitable include the water-insoluble, light-sensitive amides and esters of 2-diazo-1-naphthol-5-sulfonic acid. The adhesion of the sensitizing layer may be controlled by the addition of compatible resins, such as vinyl acetate, copolymers of vinyl acetate and crotonic acid, cellulose acetate, and the like, as well as by the addition of small amounts of active solvents for the dyed carrier layer, such as acetone, ethyl acetate, methyl Cellosolve acetate, and the like, to an essentially non-penetrating solvent.

In use, a sheet of the sensitized material is exposed beneath a positive original to a source rich in ultraviolet radiation, such as a carbon or mercury arc. The exposed sheet is then developed with a solution which removes the photoproducts and resin(s) in the irradiated areas, laying bare the dyed carrier layer. The general nature of this development process is more fully described in U.S. Patent 2,772,972. The developed sheet is then immersed in a bleaching bath. The nature of the bleach employed, and its concentration, may vary somewhat according to the dye to be bleached. However, bleaches such as bromine water, hypochlorite, hydrosulfite, and the like, are usually satisfactory. A simple test may be employed to determine whether a particular bleaching agent is suitable. When the bleaching action is complete, the sheet is rinsed in water to remove excess reagent and wiped dry. The photomechanical layer remains intact through these operations, but may be removed at this point with a solvent which dissolves it, but does not dissolve the carrier layer or the dye. Solvents suitable for this purpose are benzene, toluene, xylene, carbon tetrachloride, methyl-isobutyl ketone, and the like.

The invention will be more fully understood by reference to the accompanying drawings wherein FIGS. 1 to 7 show diagrammatically and in exaggerated cross-sectional thickness, the sequential steps involved in preparing an intermediate according to this invention.

FIG. 1 shows a base or support layer which may be film or paper of any suitable type indicated at 10. This is coated with a carrier layer 11 which, as mentioned above, preferably consists of a mixture of a copolymer of vinyl-methyl ether and maleic anhydride combined with another compatible resin which is somewhat hydrophobic.

FIG. 2 shows the same support 10, carrier layer 11, and a color layer of dye 12. This is applied, as previously mentioned, by first treating the carrier layer with an alkaline agent such as gaseous ammonia or aqueous sodium hydroxide to render it somewhat hydrophilic.

FIG. 3 shows the same layers with an additional layer 13 of sensitizing material which is to be exposed to actinic light.

FIG. 4 shows the assembly of FIG. 3 with a positive original 14 superimposed so that light may be exposed on the sensitive layer. That part of the image which is exposed is essentially decomposed at 13e.

The actinic light showing through the clear area of the original impinges on the layer 13 and this layer, where the light strikes it, decomposes.

Now referring to FIG. 5, the decomposed area (13e of FIG. 4) has been removed from the irradiated area, leaving an opening 13f, in the top layer 13. This exposes the dye layer 12. In other respects, the layers of FIG. 5 are the same as in the preceding figures.

FIG. 6 shows the results of the bleaching operation; the photomechanical layer 13, like a stencil, permits bleaching only the bared areas. The color, then, has been removed from layer 12 over area 13g and still remains in the protected areas. The layer 11 swells somewhat, partially filling the recess left by opening 13f, FIG. 5.

Finally, FIG. 7 shows the photomechanical layer 13 completely removed. Color has been bleached in the area 13g of layers 11, 12, as in FIG. 6; however, the bleaching was not effective on the color in the areas of layer protected by the stencil during the bleaching. Hence, it remains in its full color. The invention will be better understood by reference to the following examples.

#### EXAMPLE I

A preformed film of cellulose acetate manufactured by the Anasco Division of General Aniline & Film Corporation, Binghamton, New York, was coated by the reverse roll method with the following solution:

|                                                                     |     |
|---------------------------------------------------------------------|-----|
| Parts by weight of polyvinylmethyl ether maleic anhydride copolymer | 4.5 |
| Parts by weight of cellulose acetate                                | 5.5 |
| Parts by volume of acetone                                          | 140 |
| Parts by volume of ethanol                                          | 40  |
| Parts by volume of methyl Cellosolve                                | 20  |

After drying, hydrolysis was effected by immersion in a dilute solution of ammonia and the film again dried. A film prepared in this manner is hydrophilic and may be dyed with basic dyes.

A sheet of this film was immersed in a dye bath containing:

|                 |    |     |
|-----------------|----|-----|
| Water           | ml | 800 |
| Ethylene glycol | ml | 200 |
| Methylene blue  | gm | 2   |
| Diethanolamine  | ml | 2   |

for 20 seconds, rinsed with water and subsequently dried. This yielded a blue foil.

A second sheet of film was treated in a similar manner except that 3.5 grams of Magenta ABN were substituted for the 2 grams of methylene blue. This yielded a red foil.

A third sheet of film was treated in a similar manner except that 2.5 grams of Auramine O were substituted for the 2 grams of methylene blue. This yielded a yellow foil.

The dyed side of each of these three foils was then hand-sensitized with a solution containing:

|                                                                 |    |     |
|-----------------------------------------------------------------|----|-----|
| N - dihydroabietyl - 6 - diazo-5(6)-oxo-naphthalene-sulfonamide | gm | 2.0 |
| Vinylite AYAC (Bakelite)                                        | gm | 0.8 |
| Vinylite VMCH (Bakelite)                                        | gm | 0.2 |
| Acetone                                                         | ml | 15  |
| Methyl Cellosolve acetate                                       | ml | 20  |
| Methyl-isobutyl ketone                                          | ml | 65  |

After dyeing, the foils were all dried.

Each of the three dyed and sensitized foils was then exposed to actinic radiation beneath its corresponding half-tone color separation positive. The photoproducts and the decomposed resins in the irradiated portions of each exposed foil were then removed in an imagewise manner by swabbing the surface with a solution containing:

|                  |    |      |
|------------------|----|------|
| Monoethanolamine | ml | 1.5  |
| Triethanolamine  | ml | 10.0 |
| Glycerine        | ml | 25.0 |
| Ethylene glycol  | ml | 63.5 |

The red and blue developed foils were then immersed in a tray containing:

|                     |     |     |
|---------------------|-----|-----|
| Sodium bicarbonate  | gms | 20  |
| Sodium hydrosulfite | gms | 20  |
| Water               | ml  | 200 |

## 5

and the yellow foil in a tray containing:

|                                              |        |
|----------------------------------------------|--------|
| Clorox (5.25% sodium hypochlorite by weight) | ml. 50 |
| Water                                        | 200    |

The dyes were bleached to substantially total absence of color in an imagewise way within 30 seconds. The foils were then thoroughly rinsed with water and dried. The remaining portions of the upper photomechanical layer were then removed with methyl-isobutyl ketone. The unbleached portions of color were thus brought into view. When these foils were overlaid in register on one another over a white sheet of paper, a very pleasing color proof resulted.

## EXAMPLE II

A film was lacquered and hydrolyzed as in Example I. The carrier layer was then dyed in a solution containing:

|                  |         |
|------------------|---------|
| Water            | ml. 900 |
| Ethylene glycol  | ml. 100 |
| Genacryl Blue 6G | gm. 3   |
| Diethanolamine   | ml. 1   |

for about 20 seconds. It was then rinsed with water and dried. (An equal amount of Crystal Violet AX can be substituted for the Genacryl Blue 6G.) The dyed carrier layer was then sensitized as in Example I, and the coating dried. The sensitized foil was then exposed beneath a positive original and subsequently developed by swabbing it with a solution containing:

|                 |        |
|-----------------|--------|
| Diethanolamine  | ml. 15 |
| Glycerine       | ml. 15 |
| Ethylene glycol | 70     |

This treatment removed the photoproducts and resins from the carrier layer in an imagewise way. The developed foil was next immersed in a solution containing:

|                      |        |
|----------------------|--------|
| Amonia water—28° Bé. | ml. 10 |
| Water                | ml. 90 |
| Sodium hydrosulfite  | gm. 10 |

which bleached the dye in areas where the carrier layer had been laid bare. The foil was then thoroughly rinsed with water, wiped dry, and the residual sensitizing layer was removed with toluene. After a final drying, a brilliant blue, positive copy of the original on a clear background resulted.

## EXAMPLE III

A sheet of film was lacquered as in Example I. It was then immersed in a dye bath containing:

|                  |         |
|------------------|---------|
| Water            | ml. 700 |
| Ethylene glycol  | ml. 300 |
| Monoethanolamine | ml. 25  |
| Methylene Blue   | gm. 3   |

for about 30 seconds. The sheet was then rinsed and dried. In this manner, the intermediate hydrolyzing operation can be eliminated. This dyed foil can be sensitized, processed, bleached, etc. as in Example II.

## EXAMPLE IV

A preformed film of polystyrene (0.005") was coated with a solution comprising:

|                            |         |
|----------------------------|---------|
| PVM/MA                     | gm. 3.0 |
| Resin C-3, V-30 (Monsanto) | gm. 2.0 |
| Ethyl acetate              | ml. 20  |
| Methyl Cellosolve          | ml. 80  |

and thoroughly dried. The film was then immersed in a dilute ammonia solution to render the carrier layer hydrophilic and the film was dried again. The carrier layer was then dyed 20 seconds in a bath containing:

|                  |         |
|------------------|---------|
| Water            | ml. 750 |
| Ethylene glycol  | ml. 250 |
| Thioflavine TCND | gm. 5   |
| Monoethanolamine | ml. 1   |

70

65

50

55

45

35

30

15

10

## 6

rinsed with water and dried. The dyed carrier layer was then sensitized by coating it with a solution comprising:

|                                         |         |
|-----------------------------------------|---------|
| Vinylite AYAC (bakelite)                | gm. 0.8 |
| Cellulose acetate (Hercules grade LL-1) | gm. 0.2 |
| Diazo compound of the structure         | gm. 2.0 |



Milliliters

|                        |    |
|------------------------|----|
| Methyl ethyl ketone    | 20 |
| Methyl-isobutyl ketone | 70 |
| Methyl cellosolve      | 10 |

20 and dried. The sensitized foil was then exposed beneath a positive original to the radiation of a mercury arc. The exposed foil was then developed with a solution containing:

|                  |    |
|------------------|----|
| Monoethanolamine | 5  |
| Diethanolamine   | 10 |
| Glycerine        | 25 |
| Ethylene glycol  | 60 |

whereupon the photoproducts and resins in the irradiated areas were removed imagewise. The developed sheet was next immersed in a solution containing:

|        |     |
|--------|-----|
| Clorox | 100 |
| Water  | 200 |

35 until the dye had bleached imagewise and subsequently thoroughly rinsed with water and wiped dry. A treatment with methyl-isobutyl ketone removed the residual sensitizing layer. After a final drying, a yellow positive copy 40 resulted, the image portions of which were sufficiently opaque for making additional diazotype copies.

## EXAMPLE V

A sheet of the lacquered and hydrolyzed film employed in Example IV was immersed in a dye bath containing:

|                          |         |
|--------------------------|---------|
| Water                    | ml. 500 |
| Ethylene glycol          | ml. 200 |
| Diethanolamine           | ml. 1   |
| Brilliant green crystals | gm. 3   |

50 for about 20 seconds. After a rinse water to remove excessive dye solution, the film was dried. The dyed carrier layer was then sensitized by coating it with a solution comprising:

|                                          |         |
|------------------------------------------|---------|
| Vinylite AYAC (bakelite)                 | gm. 0.6 |
| Half-second butyrate (Tennessee Eastman) | gm. 0.3 |
| Vinylite VMCH (bakelite)                 | gm. 0.2 |
| Methyl-isobutyl ketone                   | ml. 70  |
| Methyl cellosolve acetate                | ml. 20  |
| Isopropyl alcohol                        | ml. 10  |
| Diazo compound of the structure          | gm. 2   |



70 and dried. A sheet of this sensitized film was then exposed, developed and processed as was done in Example IV. A bright green positive image on a clear background resulted.

## EXAMPLE VI

A sheet of film, lacquered and hydrolyzed as in Example I, was dyed in a solution containing:

|                                                                                                                            |    |     |    |
|----------------------------------------------------------------------------------------------------------------------------|----|-----|----|
| Water                                                                                                                      | ml | 750 | 5  |
| Ethylene glycol                                                                                                            | ml | 250 |    |
| Safranine Y                                                                                                                | gm | 4   |    |
| Diethanolamine                                                                                                             | ml | 2   |    |
| for about 20 seconds, and then rinsed with water. After drying, the dyed carrier was sensitized with a solution comprising |    | 10  |    |
| Vinylite AYC                                                                                                               | gm | 0.8 |    |
| Vinylite VMCH                                                                                                              | gm | 0.2 |    |
| Methyl cellosolve acetate                                                                                                  | ml | 15  | 15 |
| Acetone                                                                                                                    | ml | 20  |    |
| Methyl-isobutyl ketone                                                                                                     | ml | 65  |    |
| Diazo of the structure                                                                                                     | gm | 1.7 |    |



After drying, this sheet was exposed, developed and processed as in Example 4. A bright red positive copy on a clear background resulted.

## EXAMPLE VII

A sheet of the lacquered and hydrolyzed film as prepared in Example I was coated with a solution containing:

|                             |    |     |    |
|-----------------------------|----|-----|----|
| Water                       | ml | 85  |    |
| Ethylene glycol             | ml | 10  | 40 |
| Isopropyl alcohol           | ml | 5   |    |
| Citric acid                 | gm | 3   |    |
| Meta-hydroxyphenylurea      | gm | 3   |    |
| Thiourea                    | gm | 1   |    |
| Diazotized para-phenetidine | gm | 2   | 45 |
| Saponin                     | gm | 0.2 |    |

After drying, this sheet was subjected to moist ammonia fumes, which caused a yellow azo dye to form within the carrier layer. The carrier layer was subsequently sensitized, exposed, developed and processed as in Example IV. A yellow positive copy on a clear background resulted. This image had sufficient actinic opacity to make additional diazotype prints.

It will be obvious that variations may be made in the procedures described above and that substitution, which would occur to those skilled in the art, can be made without departing from the spirit of the invention. It is intended by the claims, which follow, to cover such varia-

tions as would occur to those skilled in the art so far as the prior art permits.

What is claimed is:

1. The process of direct positive color reproduction which comprises forming on a base, a carrier layer comprising a homogeneous mixture of a copolymer of a vinyl alkyl ether and maleic anhydride and a hydrophobic resin compatible therewith, treating said carrier layer with an alkaline material to render it more hydrophilic, dyeing said carrier layer with an intense color by imbibing it with the solution of a basic dye, covering said dyed carrier layer with a light-decomposable sensitized layer by overcoating said dyed layer with a water-insoluble adhesive resin and a light-sensitive, water-insoluble diazo oxide, exposing said sensitized layer to a colored original, removing the light-decomposed portion of said sensitized diazo oxide layer to expose a portion of the dyed carrier layer, chemically bleaching the dye from said exposed portion and stripping the remainder of said sensitized diazo oxide layer to leave a dyed positive image of said colored original.

2. The process of forming a direct positive image by diazotype reproduction which comprises forming, on a suitable base, a carrier layer composed of a mixture of a copolymer of vinyl methyl ether with maleic anhydride and of another hydrophobic resin, treating said carrier layer with a moist base to render it hydrophilic, dyeing said treated hydrophilic layer with a solution of a basic dye, applying a light-decomposable sensitized diazo oxide layer over said carrier layer, exposing the sensitized layer to actinic radiation from a colored original, removing by washing the light-decomposed portions of said sensitized diazo oxide layer to lay bare the dyed carrier layer, chemically bleaching the dye from said bare portions and causing the bleached area to swell, and stripping the undecomposed portion of said sensitized diazo oxide layer to leave a dyed positive image of said original.

3. Process according to claim 1 wherein the carrier layer comprises a mixture of vinylmethyl ether copolymerized with maleic anhydride and a hydrophobic resin.

4. Process according to claim 2 wherein the dye is closely color-matched with available printing ink, whereby the original color may be faithfully reproduced.

## References Cited

## UNITED STATES PATENTS

|           |         |                  |         |
|-----------|---------|------------------|---------|
| 2,051,603 | 8/1936  | Hruska           | 96-43   |
| 2,537,097 | 1/1951  | Slifkin          | 96-75   |
| 2,993,788 | 7/1961  | Straw et al.     | 96-13   |
| 3,091,528 | 5/1963  | Buskes           | 96-75   |
| 3,136,637 | 6/1964  | Larson           | 96-33 X |
| 3,164,468 | 1/1965  | Moskowitz et al. | 96-49   |
| 3,211,553 | 10/1965 | Ito              | 96-75   |
| 3,228,768 | 1/1966  | Straw et al.     | 96-91   |

NORMAN G. TORCHIN, Primary Examiner.

J. T. BROWN, C. BOWERS, Assistant Examiners.